



US005215840A

**United States Patent** [19]

Itami et al.

[11] **Patent Number:** **5,215,840**[45] **Date of Patent:** **Jun. 1, 1993**[54] **ELECTROPHOTOGRAPHIC  
PHOTORECEPTOR AND  
MANUFACTURING METHOD THEREOF**[75] Inventors: **Akihiko Itami; Akira Kinoshita;  
Kazumasa Watanabe, all of Hachioji,  
Japan**[73] Assignee: **Konica Corporation, Tokyo, Japan**[21] Appl. No.: **792,956**[22] Filed: **Nov. 15, 1991**[30] **Foreign Application Priority Data**

Nov. 20, 1990 [JP] Japan ..... 2-315639

[51] Int. Cl.<sup>5</sup> ..... **G03G 5/06**[52] U.S. Cl. ..... **430/58; 430/78;  
430/135**[58] **Field of Search** ..... **430/58, 78, 135**[56] **References Cited****U.S. PATENT DOCUMENTS**

|           |        |                  |       |        |
|-----------|--------|------------------|-------|--------|
| 4,981,767 | 1/1991 | Tokura et al.    | ..... | 430/78 |
| 4,994,339 | 2/1991 | Kinoshita et al. | ..... | 430/78 |
| 5,087,540 | 2/1992 | Murakami et al.  | ..... | 430/78 |

*Primary Examiner*—John Goodrow  
*Attorney, Agent, or Firm*—Jordan B. Bierman

[57] **ABSTRACT**

An electrophotographic photoreceptor and a method

for producing the same are disclosed, in which stability of coating solution of a photoreceptive layer is improved. The photoreceptor comprises a conductive support having thereon a photoreceptive layer containing a binder, a titanylphthalocyanine which has a peak in X-ray diffraction spectrum thereof by Cu-K $\alpha$  ray at a Bragg angle  $2\theta$  of  $27.2^\circ \pm 0.2^\circ$ , and a phthalocyanine derivative formed by reaction of phthalocyanine and a titanium compound represented by the following formula I or II;



wherein R<sub>1</sub>, R<sub>2</sub>, R<sub>3</sub>, R<sub>4</sub>, R<sub>5</sub> and R<sub>6</sub> are each a group capable of releasing upon reaction with said phthalocyanine.

**20 Claims, 8 Drawing Sheets**

FIG. 1



FIG. 2



FIG. 3



FIG. 4



FIG. 5



FIG. 6



FIG. 7



FIG. 8



FIG. 9



FIG. 10



FIG. II



FIG. 12



FIG. 13



FIG. 14



FIG. 15



# ELECTROPHOTOGRAPHIC PHOTORECEPTOR AND MANUFACTURING METHOD THEREOF

## FIELD OF THE INVENTION

Present invention relates to an electrophotographic photoreceptor and manufacturing method thereof.

## BACKGROUND OF THE INVENTION

In recent years, photoconductive materials are actively studied, and some of them are used as photoelectric conversion elements for electrophotographic photoreceptors, solar batteries, image sensors and the like. As such photoconductive materials, inorganic materials have been mainly used up to the present. In electrophotographic photoreceptors, for example, there have been broadly used inorganic photoreceptors provided with a photosensitive layer which contains selenium, zinc oxide, or cadmium sulfide as the primary component.

However, these inorganic photoreceptors are not always satisfactory in characteristics of photosensitivity, thermal stability, moisture resistance and durability, which are essential for electrophotographic photoreceptors used in copying machines. For example, selenium is apt to lower its properties as an electrophotographic photoreceptor for its liability to crystallization by heat or stains such as finger spots.

Further, electrophotographic photoreceptors using cadmium sulfide are low in moisture resistance and durability, and electrophotographic photoreceptors using zinc oxide are insufficient in durability.

Moreover, in the growing importance of environmental preservation, electrophotographic photoreceptors of cadmium sulfide have a defect of requiring severe control in both manufacturing and handling because of its toxicity.

For improving such disadvantages of inorganic photoconductive materials, various organic photoconductive materials have come to attract much attention in the art, and a number of approaches are being made to utilize them in the photosensitive layer of electrophotographic photoreceptors. For example, Japanese Pat. Exam. Pub. No. 10496/1975 discloses an organic photoreceptor having a photosensitive layer containing polyvinylcarbazole and trinitrofluorenone. This photoreceptor, however, is not sufficient in sensitivity and durability. Taking notice of this, there are developed electrophotographic photoreceptors of function-separated type which assign the carrier generation function and the carrier transport function to different substances separately.

These function-separated electrophotographic photoreceptors allow materials to be selected appropriately from a broad range; therefore, objective properties are obtained relatively easily, and development of an organic photoreceptor of high sensitivity and excellent durability is expected.

There are proposed various organic materials as a carrier generation material or a carrier transport material in such function-separated electrophotographic photoreceptors. And the carrier generation substance has a particularly important function which controls basic properties of a photoreceptor. As such carrier generation substances, there have been practically used photoconductive substances such as polycyclic quinones represented by dibromoanthanthrone, pyrylium compounds and eutectic complexes thereof, squarim compounds, phthalocyanine compounds and azo com-

pounds. Since the carrier generation substance is coated in the form of dispersion or solution of an organic solvent in general, a good dispersibility and high dispersion stability are required of a carrier generation substance to obtain good electrophotographic photoreceptors.

Further, a carrier generation substance having a high carrier generation efficiency is also necessary to impart a high sensitivity to an electrophotographic photoreceptor. In this connection, phthalocyanine compounds absorb much attention in recent years and are actively studied as a material to meet such necessity.

It is known that characteristics of the phthalocyanine compound including spectrum and photoconductivity vary according to types of central metals and crystal forms. For example, it is reported, in "Senryo to Yakuhin" (Dyes and Related Chemicals) by M. Sawata, 24 (6), p. 122 (1979), that copper phthalocyanine has three crystal forms:  $\alpha$ ,  $\beta$ ,  $\gamma$  and  $\epsilon$ , and that its electrophotographic characteristics vary depending upon the crystal forms.

Titanylphthalocyanine, which is particularly interested recently, is also reported to have four crystal forms of types A, B, C and Y. Titanylphthalocyanine of type A described in Japanese Pat. O.P.I. Pub. No. 67094/1987, type B in Japanese Pat. O.P.I. Pub. No. 239248/1986 and type C in Japanese Pat. O.P.I. Pub. No. 256865/1987 are still insufficient in electrophotographic sensitivity and durability.

Titanylphthalocyanine of type Y made known recently in "Japan Hardcopy '89" by Kinoshita et al., EP 26 (1989) has a high sensitivity; for utilizing its high characteristics practically by making its dispersion stably and finely, it is essential to develop a new technique to prepare its dispersion.

## SUMMARY OF THE INVENTION

The object of the present invention is to provide an electrophotographic photoreceptor excellent in stability of the coating solution and manufacturing method thereof.

The above object of the invention is attained by an electrophotographic photoreceptor containing, as the carrier generation substance, a titanylphthalocyanine (hereinafter referred to as titanylphthalocyanine of the invention) having a characteristic peak at a Bragg angle  $2\theta$  of  $27.2 \pm 0.2^\circ$ , preferably a titanylphthalocyanine having characteristic peaks at Bragg angles  $2\theta$  of  $9.5 \pm 0.2^\circ$ ,  $24.1 \pm 0.2^\circ$  and  $27.2 \pm 0.2^\circ$  in an X-ray diffraction spectrum given by a Cu-K $\alpha$ -ray (wavelength: 1.541 Å) and a phthalocyanine derivative (hereinafter referred to as phthalocyanine derivative of the invention) prepared by reacting a phthalocyanine compound with a titanium compound represented by the following formula I or II.



In the formulas, R<sub>1</sub> to R<sub>6</sub> each represent a group capable of being released upon reaction with the titanypthalocyanine.

Titanypthalocyanine of the invention is represented by the following formula III. formula III



In the formula, X<sup>1</sup>, X<sup>2</sup>, X<sup>3</sup> and X<sup>4</sup> each represent a hydrogen or halogen atom, or an alkyl or alkoxy group; n, m, l and k each represent an integer of 0 or 4.

The X-ray diffraction spectrum was measured under the following conditions, and the peak means a clear projection of sharp angle which differs from noises.

|                |           |
|----------------|-----------|
| X-ray vessel   | Cu        |
| Voltage        | 40.0 KV   |
| Current        | 100 mA    |
| Start angle    | 6.0 deg.  |
| Stop angle     | 35.0 deg. |
| Step angle     | 0.02 deg. |
| Measuring time | 0.50 sec. |

#### BRIEF DESCRIPTION OF THE DRAWING

FIGS. 1 to 6 are sectional views showing typical examples of the layer configuration of the photoreceptor according to the invention.

FIGS. 7 to 11 are X-ray diffraction spectral maps of titanypthalocyanines used in the invention.

FIGS. 12 and 14 are an absorption spectrum and IR spectrum of the phthalocyanine derivative obtained in synthesis 1, respectively.

FIGS. 13 and 15 are an absorption spectrum and IR spectrum of the phthalocyanine derivative obtained in synthesis 2, respectively.

#### DETAILED DESCRIPTION OF THE INVENTION

Various methods can be used to synthesize the titanypthalocyanine used in the invention, but typically it is synthesized according to the following reaction formula (1) or (2).



In the formulas, R<sub>1</sub> to R<sub>4</sub> each represent a group capable of being released upon the above reaction.

The titanypthalocyanine obtained as above can be converted into the crystal form used in the invention by subjecting it to the following treatment.

For example, a titanypthalocyanine of any crystal form is dissolved in a concentrated sulfuric acid, and the sulfuric acid solution is poured into water to precipitate crystals, which are then filtered off. In this process, the titanypthalocyanine is converted into an amorphous state.

Subsequently, this amorphous titanypthalocyanine is treated with an organic solvent in the presence of moisture to obtain the crystal form used in the invention. Usable organic solvent includes aliphatic hydrocarbons, aromatic hydrocarbons, halogenized hydrocarbons, ketones, esters, ethers, alcohols and heterocyclic compounds. But the method for converting the crystal form is not limited to the foregoing.

The following is an example of synthesis of titanypthalocyanine of the invention. Syntheses example of titanypthalocyanine

To a mixture of 29.2 g of 1,3-diiminoisoindoline and 200 ml of  $\alpha$ -chloronaphthalene, 20.4 g of titanium tetrabutoxide was added and reacted at 180° C. for 5 hours in nitrogen atmosphere. The reacted product was stood for cooling and precipitate was separated by filtration. The precipitate was washed with  $\alpha$ -chloronaphthalene for several times and further washed with 2% hydrochloric acid followed by washing with water. The precipitate was further washed with alcohol and dried. Thus 26.2 g of crystal was obtained.

At a temperature lower than 5° C., 5 g of the crystal was dissolved in 250 g of concentrated sulfuric acid. After stirring for 1 hour, the solution was poured into 5 liter of water to precipitate crystal. The crystal was filtered off and washed for several times with deionized water. Wet paste thus obtained was stirred for 5 hours with 50 g of 1,2-dichloroethane and precipitate was filtered off. The precipitate was washed with methanol for several times and dried. After drying 4.6 g of blue colored crystal of titanypthalocyanine was obtained. Thus obtained titanypthalocyanine has a clear peak at 27.2° ± 0.2° of Bragg angle 2 $\theta$  of X-ray diffraction spectrum thereof as shown in FIG. 7.

The phthalocyanine derivative of the invention is prepared by making a phthalocyanine react with a titanium compound represented by formula I or II, in an inactive solvent such as  $\alpha$ -chloronaphthalene at a high temperature not less than 100° C. Though the type of phthalocyanine is not particularly limited, trivalent or tetravalent metal phthalocyanines are preferred. Examples thereof are metal phthalocyanines containing aluminum, gallium, indium, titanium, vanadium, zirconium, tin, manganese, silicon or germanium. Of these phthalocyanines, substituted or unsubstituted titanypthalocyanine and vanadylphthalocyanine are particularly preferred.

As the titanium compound, any of the compounds represented by formula I or II may be used.

As the group capable of being released represented by R<sub>1</sub> to R<sub>4</sub> of formula I and R<sub>1</sub> to R<sub>6</sub> of formula II, the following

groups are preferable: —R, —OR, —SR, —OSO<sub>2</sub>R, —OCOR,



wherein R is a hydrogen atom, an

alkyl group, an alkenyl group, an aralkyl group, an acyl group, an aryloxy group or a heterocyclic group, these groups may have a substituent and are allowed to bond with each other to form a ring. In the groups having a plurality of R's, groups represented by each of the R's may be the same or different from each other. Among the above-mentioned group capable of releasing, an alkoxy group is most preferable. There can be used commercially available alkoxy titans such as Plenact manufactured by Ajinomoto Co. Ltd. The following 20 are examples of the titanium compound.

- (1)  $\text{Ti}(\text{OC}_2\text{H}_5)_4$
- (2)  $\text{Ti}(\text{OC}_3\text{H}_7-(n))_4$
- (3)  $\text{Ti}(\text{OC}_3\text{H}_7-(i))_4$
- (4)  $\text{Ti}(\text{OC}_4\text{H}_9-(n))_4$
- (5)  $\text{Ti}(\text{OC}_4\text{H}_9-(t))_4$
- (6)



(7)



(8)



(9)



(10)



(11)



(12)



(13)



25 The electrophotographic photoreceptor according to the invention is formed by coating, on a substrate, a coating solution which comprises a binder solution dispersing therein the titanylphthalocyanine of the invention and a soluble phthalocyanine. There is no particular limitation on the method for incorporating a phthalocyanine of the invention in a coating solution of the titanylphthalocyanine having a specific crystal form of the invention. For example, these compounds may be mixed in a solid state, or a phthalocyanine may be added 35 to a dispersion of the titanylphthalocyanine.

Further, these may be mixed by steps of making up respective phthalocyanines into uniformly dissolved states, allowing them to form mixed crystals or complexes, and then dispersing them.

40 The mixing ratio of a phthalocyanine of the invention to a titanylphthalocyanine of the invention is usually 0.0001 wt% to 100 wt%, desirably 0.001 to 50 wt% and more desirably 0.01 to 20 wt%.

In addition to these phthalocyanines, there may be 45 contained other photoconductive substances in the electrophotographic photoreceptor of the invention.

Examples of such other photoconductive substances include titanylphthalocyanines different in crystal forms from the titanylphthalocyanine of the invention, 50 such as types A, B and C, amorphous titanylphthalocyanines, and mixtures thereof including a mixture of types A and B; other phthalocyanine compounds; naphthalocyanine compounds; porphyrin compounds; azo compounds; polycyclic quinone compounds represented by dibromoanthanthrone; pyrylium compounds 55 and eutectic complexes thereof; and squarim compounds.

In the electrophotographic photoreceptor of the invention, a carrier transport substance may be used 60 jointly with the carrier generation substance.

While various substances can be used as the carrier transport substance, typical ones are nitrogen-containing heterocyclic nuclei such as oxazole, oxaziazone, thiazole, thiaziazole and compounds having a condensed ring thereof; polyarylalkane compounds; pyrazoline compounds; hydrazone compounds; triazoleamine compounds; styryl compounds; polys(bis)styryl compounds; styryltriphenylamine com-

pounds;  $\beta$ -phenylstyryltriphenylamine compounds; butadiene compounds; hexatriene compounds; carbazole compounds; and condensed polycyclic compounds.

Typical examples of such carrier transport substances can be seen in Japanese Pat. O.P.I. Pub. No. 107356/1986; among them, representative ones are illustrated below.



-continued



(8)



(9)



(10)



(11)



(12)



(13)



(14)

-continued



-continued



(22)

As the layer configuration of photoreceptors, various types are known in the art.

While the present invention can use any of the layer configurations, it is preferable that the photoreceptor be formed into a function-separated photoreceptor of laminated-type or dispersed-type shown in FIGS. 1 to 6. The layer configuration shown in FIG. 1 is given by forming, on electroconductive support 1, carrier generation layer 2 containing a titanylphthalocyanine of the invention and a phthalocyanine derivative, and laminating thereon carrier transport layer 3 to form photosensitive layer 4. In FIG. 2, carrier generation layer 2 and carrier transport layer 3 are provided in the reverse order to form photosensitive layer 4'. In FIG. 3, intermediate layer 5 is provided between photoconductive layer 4, and electroconductive support 1 shown in the layer configuration of FIG. 1. The layer configuration of FIG. 5 is given by forming photosensitive layer 4'' containing the carrier generation substance of the invention 6 and carrier transport substance 7. In FIG. 6, intermediate layer 5 is provided between said photosensitive layer 4'' and electroconductive support 1. In the layer configurations of FIGS. 1 to 6, a protective layer may be provided on the uppermost layer.

A useful method of forming a photosensitive layer is to coat a solution dissolving or dispersing a carrier generation substance or a carrier transport substance singly or together with a binder and additives.

However, carrier generation substances of the invention are generally low in solubility. Accordingly, it is advantageous to coat a dispersion prepared by dispersing a carrier generation substance as fine particles in a suitable dispersion medium with a dispersing apparatus such as a supersonic disperser, ball mill, sand mill or homogenizer. In this case, a binder and other additives are generally added to such a dispersion.

As a solvent or dispersing medium used in forming a photosensitive layer, there may be employed various compounds such as butylamine, ethylenediamine, N,N-dimethylformamide, acetone, methyl ethyl ketone, methyl isopropyl ketone, methyl isobutyl ketone, cyclohexanone, 4-methoxy-4-methyl-2-pentanone, tetrahydrofuran, dioxane, ethyl acetate, butyl acetate, t-butyl acetate, methyl cellosolve, ethyl cellosolve, butyl cellosolve, ethylene glycol dimethyl ether, toluene, xylene, acetophenone, chloroform, dichloromethane, dichloroethane, trichloroethane, methanol, ethanol, propanol and butanol.

The binder used in forming a carrier generation layer or a carrier transport layer may be arbitrarily selected, but hydrophobic high polymers having a film forming capability are preferred. Examples of these polymers are illustrated below.

Polycarbonate resins  
Polycarbonate Z resins

- 15 Acrylic resins  
Methacrylic resins  
Polyvinyl chlorides  
Polyvinylidene chlorides  
Polystyrenes  
20 Styrene-butadien copolymers  
Polyvinyl acetates  
Polyvinyl formals  
Polyvinyl butyrals  
Polyvinyl acetals  
25 Polyvinylcarbazoles  
Styrene-alkyd resins  
Silicone resins  
Silicone-alkyd resins  
Silicone-butylal resins  
30 Polyesters  
Polyurethanes  
Polyamides  
Epoxy resins  
Phenolic resins  
35 Vinylidene chloride-acrylonitrile copolymers  
Vinyl chloride-vinyl acetate copolymer  
Vinyl chloride-vinyl acetate-maleic anhydride copolymers

The addition ratio of the carrier generation substance, i.e. a titanylphthalocyanine of the invention, to the binder is desirably 10 to 600 wt% and more desirably 50 to 400 wt%. The addition ratio of the carrier transport substance to the binder is desirably 10 to 500 wt%. The thickness of the carrier generation layer is 0.01 to 20  $\mu$ m and preferably 0.05 to 5  $\mu$ m. The thickness of the carrier transport layer is 1 to 100  $\mu$ m and preferably 5 to 30  $\mu$ m.

The above photosensitive layer may contain an electron accepting substance for enhancing the sensitivity, decreasing the residual voltage and lessening the fatigue in a repeated use. Examples of such electron accepting substances include succinic anhydride, maleic anhydride, dibromosuccinic anhydride, phthalic anhydride, tetrachlorophthalic anhydride, tetrabromophthalic anhydride, 3-nitrophthalic anhydride, 4-nitrophthalic anhydride, pyromellitic anhydride, mellitic anhydride, tetracyanoethylene, tetracyano quinodimethane, o-dinitrobenzene, m-dinitrobenzene, 1,3,5-trinitrobenzene, p-nitrobenzonitrile, picryl chloride, quinonechloroimide, chloranil, bromanil, dichlorodicyano-p-benzoquinone, anthraquinone, dinitroanthraquinone, 9-fluorenylidene-malonodinitrile, polynitro-9-fluorenylidene-malonodinitrile, picric acid, o-nitrobenzoic acid, p-nitrobenzoic acid, 3,5-dinitrobenzoic acid, pentafluorobenzoic acid, 5-nitrosalicylic acid, 3,5-dinitrosalicylic acid, phthalic acid, mellitic acid and other compounds having a large electron affinity. The addition amount of the electron accepting substance is desirably 0.01 to 200 parts, more desirably 0.1 to 100 parts by

weight per 100 parts by weight of the carrier generation substance.

In order to improve the preservability, durability and anti-environmental dependency, the photosensitive layer may contain deterioration inhibitors such as anti-oxidants and light-stabilizers. The compounds used for such purposes are, for example, chromanol derivatives and ethers or esters thereof such as tocopherol; poly-arylalkane compounds; hydroquinone derivatives and mono or dithers thereof; benzophenone derivatives; benzotriazole derivatives; thioether compounds; phosphonates; phosphites; phenylenediamine derivatives; phenol compounds; hindered phenol compounds; straight chain amines; cyclic amines; and hindered amines. Typical examples of particularly useful compounds are hindered phenol compounds such as those available by names of Irganox 1010, Irganox 565 (products of Ciba Geigy), Sumilizer BHT, Sumilizer MDP (products of Sumitomo Chemical) and hindered amine compounds such as those available by names of Sanol LS-2626 and Sanol LS-622LD (products of Sankyo).

As the binder for the intermediate layer and protective layer, binders used in the above carrier generation layer and carrier transport layer can be employed. In addition, there may be used other types of binders such as nylon resins; ethylene-type resins including ethylene-vinyl acetate copolymers, ethylene-vinyl acetate-maleic anhydride copolymers and ethylene-vinyl acetate-methacrylic acid copolymers; polyvinyl alcohols; and cellulose derivatives. Curable binders which utilize a thermosetting or chemical curing function of melamine, epoxides or isocyanates may also be used.

Electroconductive supports suitable for the invention are metal plates and metal drums, as well as ones prepared by forming a thin film of an electroconductive polymer, electroconductive compound such as iridium oxide or metal such as aluminium or palladium, on a paper or plastic film substrate by means of coating, deposition or lamination.

## EXAMPLES

### Synthesis Example 1

In a stream of nitrogen, 5 g of titanylphthalocyanine, 60 g of titanium tetrabutoxide and 100 ml of quinoline were mixed and refluxed under heating and stirring for 45 8 hours. After that, the reaction liquor was allowed to cool to room temperature, and the crystals formed were filtered off. The crystals were washed with methanol and then stirred in a 2% aqueous hydrochloric acid to remove an excessive amount of alkoxy titane and decomposed materials. After repeating rinsing with water and washing with methanol several times, there were obtained 1.5 g of green crystals. The absorption spectrum and IR spectrum of the crystals are shown in FIGS. 12 and 14, respectively. This compound showed a characteristic spectrum having two absorption maxima at 670 nm and 695 nm. And as apparent from the IR spectrum, it was confirmed to be a titanylphthalocyanine derivative. The titanylphthalocyanine derivative thus obtained is referred to as phthalocyanine derivative 1.

### Synthesis Example 2

The same reaction as that in synthesis 1 was carried out, except that tetraphenoxy titanylphthalocyanine was used instead of titanylphthalocyanine. After cooling the reaction to room temperature, it was poured into 1.5 liter of methanol and stirred. The crystal formed

were filtered off and treated with a 2% aqueous hydrochloric acid as in synthesis 1, followed by rinsing with water and washing with methanol, so the 2.0 g of bluish green crystals were obtained. The absorption spectrum and IR spectrum of the crystals are shown in FIGS. 13 and 15, respectively. The titanylphthalocyanine derivative thus obtained is referred to as phthalocyanine derivative 2.

### Example 1-1

A dispersion was prepared by dispersing, with a sand mill, 1 part of titanylphthalocyanine of the invention shown in FIG. 7 and having a characteristic peak at a Bragg angle ( $2\theta$ ) of 27.2°, 0.01 part of phthalocyanine derivative 1, 1 part of silicone resin (KR-5240, 15% xylene-butanol solution, product of Shin-Etsu Chemical) as the binder resin and 100 parts of methyl ethyl ketone as the dispersion medium. The dispersion was coated on an aluminium-deposited polyester base using a wire bar to form a 0.2- $\mu\text{m}$  thick carrier generation layer.

Next, there was coated thereon, with a blade coater, a solution dissolving 1 part of exemplified carrier transport substance (1), 1.3 parts of polycarbonate resin (Eupiron Z200 made by Mitsubishi Gas Chemical) and a small amount of silicone oil (KF-54 made by Shin-Etsu Chemical) in 10 parts of 1,2-dichloroethane to form a 20- $\mu\text{m}$  thick carrier transport layer. The photoreceptor prepared as above is referred to as sample 1.

### Example 1-2

A photoreceptor was prepared in the same procedure as in Example 1-1, except that the dispersion obtained in Example 1-1 was allowed to stand in the dark at 60° C. for 1 month and then used. This is referred to as sample 1'.

### Example 2-1

40 A photoreceptor was prepared in the same procedure as in Example 1-1, except that phthalocyanine derivative 2 was used instead of phthalocyanine 1. This is referred to as sample 2.

### Example 2-2

A photoreceptor was prepared in the same procedure as in Example 2-1, except that the dispersion obtained in Example 2-1 was allowed to stand in the dark for 1 month as in Example 1-2 and then used. This is referred to as sample 2'.

### Example 3-1

55 A photoreceptor was prepared in the same procedure as in Example 1-1, except that phthalocyanine derivative 1 was used in amount of 0.05 part instead of 0.01 part. This is referred to as sample 3.

### Example 3-2

A photoreceptor was prepared in the same procedure as in Example 3-1, except that the dispersion obtained in Example 3-1 was allowed to stand in the dark for 1 month as in Example 1-2 and then used. This is referred to as sample 3'.

### Example 4-1

A photoreceptor was prepared in the same procedure as in Example 1-1, except that the titanylphthalocyanine shown in FIG. 11 was used instead of the titanylph-

thalocyanine shown in FIG. 7 and that exemplified carrier transport substance (22) was used instead of exemplified carrier transport substance (1). This is referred to as sample 4.

### Example 4-2

A photoreceptor was prepared after allowing the dispersion obtained in Example 4-1 to stand in the dark for 1 month as in Example 1-2. This is referred to as sample 4'.

### Comparison 1—1

A photoreceptor was prepared in the same procedure as in Example 1-1, except that phthalocyanine derivative 1 was not used. This is referred to as comparative sample 1.

### Comparison 1-2

A photoreceptor was prepared after allowing the dispersion obtained in Comparison 1-1 to stand in the dark for 1 month as in Example 1-2. This is referred to as comparative sample 1'.

## Evaluation 1

The samples prepared as above were subjected to the following evaluation with a paper analyzer Model EPA-8100 (product of Kawaguchi Electric). First, each sample was subjected to corona electrification for 5 seconds at  $-80 \mu\text{A}$  to determine the surface potential immediately after the electrification  $V_a$  and the surface potential after allowing the sample stand for 5 seconds  $V_i$ . Subsequently, the sample was exposed under a condition giving it a surface illumination intensity of 2 (lux) to determine the exposure  $E_2$  necessary to make the surface potential  $\frac{1}{2} V_i$  and the exposure  $E_{600/100}$  necessary to drop the surface potential from  $-600 \text{ V}$  to  $-100 \text{ V}$ . Further, the dark attenuation factor  $D$  was determined from the equation  $D = 100(v_a - V_i)/V_a (\%)$ . The results are shown in Table 1.

TABLE 1

| Sample No.            | V <sub>a</sub><br>(V) | V <sub>i</sub><br>(V) | D<br>(%) | E <sub>½</sub><br>(lux · sec) | E <sub>600/100</sub><br>(lux · sec) |
|-----------------------|-----------------------|-----------------------|----------|-------------------------------|-------------------------------------|
| Sample 1              | -1175                 | -960                  | 18.3     | 0.33                          | 0.38                                |
| Sample 1'             | -1150                 | -935                  | 18.7     | 0.36                          | 0.40                                |
| Sample 2              | -1160                 | -940                  | 19.0     | 0.35                          | 0.39                                |
| Sample 2'             | -1160                 | -935                  | 19.4     | 0.36                          | 0.41                                |
| Sample 3              | -1140                 | -890                  | 21.9     | 0.38                          | 0.42                                |
| Sample 3'             | -1135                 | -885                  | 22.0     | 0.38                          | 0.43                                |
| Sample 4              | -1190                 | -980                  | 17.6     | 0.32                          | 0.34                                |
| Sample 4'             | -1180                 | -965                  | 18.2     | 0.35                          | 0.38                                |
| Comparative sample 1  | -1185                 | -965                  | 18.6     | 0.33                          | 0.39                                |
| Comparative sample 1' | -1080                 | -780                  | 27.8     | 0.47                          | 0.62                                |

It can be seen from these results that each coating solution of the invention has an excellent stability.

### Example 5

A 0.1- $\mu\text{m}$  thick intermediate layer of vinyl chloride-vinyl acetate copolymer (Ethlec MF-10 made by Sekisui Chemical) was formed on an aluminium drum. Separately, a dispersion was prepared by steps of grinding 1 part of titanylphthalocyanine of the invention shown in FIG. 7 and 0.01 part of phthalocyanine derivative 1 in a ball mill, adding thereto a mixture of 3 parts of polycarbonate resin (Panlite L-1250), 15 parts of monochlorobenzene and 35 parts of 1,2-dichloroethane, followed by dispersing. After further adding 2 parts of carrier transport substance (1) to the dispersion, it was coated on the

foregoing intermediate layer by the dipping method and dried, so that a 20- $\mu\text{m}$  thick photosensitive layer was formed. The photoreceptor prepared as above is referred to as sample 5.

In addition, a photoreceptor was prepared after allowing the above dispersion to stand for 1 month as in Example 1-2. This is referred to as sample 5'.

## Comparison 2

A photoreceptor was prepared in the same manner as in Example 5, except that phthalocyanine derivative 1 was not used. This photoreceptor is referred to as comparative sample 2, and a photoreceptor prepared after allowing the dispersion to stand for 1 month is referred to as comparative sample 2'. Samples prepared as above were evaluated in the same way as in evaluation 1, except that a positive polarity was used as the electrification polarity. The results are shown in Table 2.

TABLE 2

| Sample No.               | V <sub>a</sub><br>(V) | V <sub>i</sub><br>(V) | D<br>(%) | E <sub>½</sub><br>(lux · sec) | E <sub>600/100</sub><br>(lux · sec) |
|--------------------------|-----------------------|-----------------------|----------|-------------------------------|-------------------------------------|
| Sample 5                 | 1310                  | 1050                  | 19.8     | 0.42                          | 0.54                                |
| Sample 5'                | 1300                  | 1030                  | 20.8     | 0.43                          | 0.57                                |
| Comparative<br>sample 2  | 1305                  | 1045                  | 19.9     | 0.42                          | 0.55                                |
| Comparative<br>sample 2' | 1220                  | 890                   | 27.0     | 0.49                          | 0.73                                |

The coating solutions of the invention exhibited good preservabilities in the positively electrifying evaluation, too.

**What is claimed is:**

1. An electrophotographic photoreceptor comprising a conductive support having thereon a photoreceptive layer containing a binder, a titanylphthalocyanine represented by the following formula III, which has a peak in X-ray diffraction spectrum thereof by Cu-K $\alpha$  ray at a Bragg angle  $2\theta$  of  $27.2^\circ \pm 0.2^\circ$ , and a phthalocyanine derivative formed by reaction of a phthalocyanine and a titanium compound represented by the following formula I or II:



wherein R<sub>1</sub>, R<sub>2</sub>, R<sub>3</sub>, R<sub>4</sub>, R<sub>5</sub> and R<sub>6</sub> are each a group capable of releasing upon reaction with said phthalocyanine;



wherein  $X^1$ ,  $X^2$ ,  $X^3$  and  $X^4$  are each a hydrogen atom, a halogen atom, an alkyl group or an alkoxy group; and  $n$ ,  $m$ ,  $l$  and  $k$  are each an integer of 0, 1, 2, 3 to 4.

2. A photoreceptor of claim 1, wherein said group represented by  $R_1$ ,  $R_2$ ,  $R_3$  or  $R_4$  in formula I are each a  $-R$  group, a  $-OR$  group, a  $-SR$  group, a  $-OSO_2R$  group, a  $-OCOR$



group, wherein  $R$  is a hydrogen atom, an alkyl group, an alkenyl group, an aralkyl group, an acyl group, an aryloyl group or a heterocyclic group, these groups may have a substituent and are allowed to bond with each other to form a ring, in the groups having a plurality of  $Rs$ , groups represented by each of the  $Rs$  may be the same or different.

3. A photoreceptor of claim 2, wherein said group represented by  $R_1$ ,  $R_2$ ,  $R_3$  or  $R_4$  in formula I are each an alkoxy group.

4. A photoreceptor of claim 1, wherein said group represented by  $R_1$ ,  $R_2$ ,  $R_3$ ,  $R_4$ ,  $R_5$  or  $R_6$  in formula II are each a  $-R$  group, a  $-OR$  group, a  $-SR$  group, a  $-OSO_2R$  group, a  $-OCOR$



group, wherein  $R$  is a hydrogen atom, an alkyl group, an alkenyl group, an aralkyl group, an acyl group, an aryloyl group or a heterocyclic group, these groups may have a substituent and are allowed to bond with

each other to form a ring, in the groups having a plurality of  $Rs$ , groups represented by each of the  $Rs$  may be the same or different.

5. A photoreceptor of claim 4, wherein said group represented by  $R_1$ ,  $R_2$ ,  $R_3$ ,  $R_4$ ,  $R_5$  or  $R_6$  in formula II are each an alkoxy group.

6. A photoreceptor of claim 1, wherein said titanylphthalocyanine has peaks in X-ray diffraction spectrum at Bragg angles  $2\theta$  of  $9.5^\circ \pm 0.2^\circ$ ,  $24.1^\circ \pm 0.2^\circ$  and  $27.2^\circ \pm 0.2^\circ$ .

7. A photoreceptor of claim 1, wherein said phthalocyanine derivative is contained in said photoreceptive layer in a ratio of from 0.001% to 50% of said titanylphthalocyanine by weight.

15 8. A photoreceptor of claim 7, wherein said phthalocyanine derivative is contained in said photoreceptive layer in a ratio of from 0.01% to 20% of said titanylphthalocyanine by weight.

20 9. A photoreceptor of claim 1, wherein said photoreceptor further comprises a carrier transport layer comprising a binder and a carrier transpot substance.

25 10. An electrophotographic photoreceptor comprising a conductive support having thereon a photoreceptive layer containing a binder, a titanylphthalocyanine represented by the following formula III, which has peaks in X-ray diffraction spectrum thereof by Cu-K $\alpha$  ray at a Bragg angle  $2\theta$  of  $9.5^\circ \pm 0.2^\circ$ ,  $24.1^\circ \pm 0.2^\circ$  and  $27.2^\circ \pm 0.2^\circ$  and a phthalocyanine derivative formed by reaction of a phthalocyanine and a titanium compound represented by the following formula I or II;



wherein  $R_1$ ,  $R_2$ ,  $R_3$ ,  $R_4$ ,  $R_5$  and  $R_6$  are each an alkoxy group;



50 wherein  $X^1$ ,  $X^2$ ,  $X^3$  and  $X^4$  are each a hydrogen atom, a halogen atom, an alkyl group or an alkoxy group; and  $n$ ,  $m$ ,  $l$  and  $k$  are each an integer of 0, 1, 2, 3 to 4.

55 65 11. A method for producing an electrophotographic photoreceptor comprising steps of dispersing a titanylphthalocyanine represented by the following formula III, which has a peak in X-ray diffraction spectrum thereof by Cu-K $\alpha$  ray at a

Bragg angle  $2\theta$  of  $27.2^\circ \pm 0.2^\circ$ , and a phthalocyanine derivative formed by reaction of phthalocyanine; and a titanium compound represented by the following formula I or II, in a solution of a binder to form a coating solution; and

coating said coating solution on a conductive support;



wherein  $R_1$ ,  $R_2$ ,  $R_3$ ,  $R_4$ ,  $R_5$  and  $R_6$  are each a group capable of releasing upon reaction with said phthalocyanine;



wherein  $X^1$ ,  $X^2$ ,  $X^3$  and  $X^4$  are each a hydrogen atom, a halogen atom, an alkyl group or an alkoxy group; and  $n$ ,  $m$ ,  $l$  and  $k$  are each an integer of 0, 1, 2, 3 to 4.

12. A method of claim 11, wherein said group represented by  $R_1$ ,  $R_2$ ,  $R_3$  or  $R_4$  in formula I are each a  $-R$  group, a  $-OR$  group, a  $-SR$  group, a  $-OSO_2R$  group, a  $-OCOR$



group, wherein  $R$  is a hydrogen atom, an alkyl group, an alkenyl group, an aralkyl group, an acyl group, an aryloxy group or a heterocyclic group, these groups may have a substituent and are allowed to bond with each other to form a ring, in the groups having a plurality of  $R$ s, groups represented by each of the  $R$ s may be the same or different.

13. A method of claim 12, wherein said group represented by  $R_1$ ,  $R_2$ ,  $R_3$  or  $R_4$  in formula I are each an alkoxy group.

14. A method of claim 11, wherein said group represented by  $R_1$ ,  $R_2$ ,  $R_3$ ,  $R_4$ ,  $R_5$  or  $R_6$  in formula II are each a  $-R$  group, a  $-OR$  group, a  $-SR$  group, a  $-OSO_2R$  group, a  $-OCOR$



group, wherein  $R$  is a hydrogen atom, an alkyl group, an alkenyl group, an aralkyl group, an acyl group, an aryloxy group or a heterocyclic group, these groups may have a substituent and are allowed to bond with each other to form a ring, in the groups having a plurality of  $R$ s, groups represented by each of the  $R$ s may be the same or different.

15. A method of claim 14, wherein said group represented by  $R_1$ ,  $R_2$ ,  $R_3$ ,  $R_4$ ,  $R_5$  or  $R_6$  in formula II are each an alkoxy group.

16. A method of claim 11, wherein said titanylphthalocyanine has peaks in X-ray diffraction spectrum at Bragg angles  $2\theta$  of  $9.5^\circ \pm 0.2^\circ$ ,  $24.1^\circ \pm 0.2^\circ$  and  $27.2^\circ \pm 0.2^\circ$ .

17. A method of claim 16, wherein said phthalocyanine derivative is contained in said photoreceptive layer in a ratio of from 0.001% to 50% of said titanylphthalocyanine by weight.

18. A method of claim 17, wherein said phthalocyanine derivative is contained in said photoreceptive layer in a ratio of from 0.01% to 20% of said titanylphthalocyanine by weight.

19. A method of claim 11, wherein said photoreceptor further comprises a carrier transport layer comprising a binder and a carrier transpot substance.

20. A method for producing an electrophotographic photoreceptor comprising steps of dispersing a titanylphthalocyanine represented by the following formula III, which has peaks in X-ray diffraction spectrum thereof by  $Cu-K\alpha$  ray at a Bragg angle  $2\theta$  of  $9.5^\circ \pm 0.2^\circ$ ,  $24.1^\circ \pm 0.2^\circ$  and  $27.2^\circ \pm 0.2^\circ$ , and a phthalocyanine derivative formed by reaction of phthalocyanine; and a titanium compound represented by the following formula I or II, in a solution of a binder to form a coating solution; and coating said coating solution on a conductive support;





wherein R<sub>1</sub>, R<sub>2</sub>, R<sub>3</sub>, R<sub>4</sub>, R<sub>5</sub> and R<sub>6</sub> are each an alkoxy 10

### GROUP:

20

wherein  $X^1$ ,  $X^2$ ,  $X^3$  and  $X^4$  are each a hydrogen atom, a halogen atom, an alkyl group or an alkoxy group; and  $n$ ,  $m$ ,  $l$  and  $k$  are each an integer of 0, 1, 2, 3 to 4.

an integer or

23

30

35

40

45

50

2

8

65